

Patented Dec. 9, 1924.

1,518,931

# UNITED STATES PATENT OFFICE.

HAROLD I. HUEY, OF SAYLESVILLE, RHODE ISLAND, ASSIGNOR TO SAYLES FINISHING PLANTS, INC., OF SAYLESVILLE, RHODE ISLAND, A CORPORATION OF RHODE ISLAND.

## PROCESS FOR PRODUCING WOOLLIKE EFFECTS UPON COTTON FABRICS.

No Drawing.

Application filed May 31, 1922. Serial No. 564,979.

To all whom it may concern:

Be it known that I, HAROLD I. HUEY, a citizen of the United States, residing at Saylesville, in the county of Providence and State of Rhode Island, have invented an Improvement in Processes for Producing Woollike Effects Upon Cotton Fabrics, of which the following description is a specification.

10 This invention relates to processes for producing wool-like or "challie" effects in cotton fabrics.

The fact that a cotton fabric treated with concentrated sulphuric acid undergoes a 15 chemical and structural change and assumes a parchment-like appearance was made known by Mercer in 1844, who obtained the effects by treatment of the fabric with sulphuric acid of a concentration of from 49.5° to 53.5° Bé. The action of sulphuric acid is also known to be more intense when the 20 cotton fabric has been previously mercerized and the concentration is over 50½° Bé.

Wool-like effects have heretofore been 25 produced in cotton fabrics by subjecting the fabric for some minutes to the action of sulphuric acid of a concentration of from 49° to 51° Bé. and also like effects have been produced by repeated treatment of the cotton fabric with sulphuric acid of from 49° to 50½° Bé. and an alkali lye. Regulation 30 of temperature to something like 0° C. has still further been known to give the desired finish.

35 To secure the desired results or wool-like effects in cotton fabric in any case has heretofore required nicety of control of the sulphuric acid concentration, since variation in this respect causes marked variations in the 40 character and appearance of the product. One of the purposes of the present invention, therefore, is to provide a process for the production of wool-like or challie effects in cotton fabrics in which a wide range 45 of variation in the concentration of the acid employed may be possible without material variation in the resulting product.

Where the concentration of the sulphuric acid must be maintained substantially constant and at a substantially fixed point or between very narrow limits, the watchful care of skilled operatives is required to secure the desired result and avoid damage or variation in the fabric under treatment.

One of the important features of the present 55 invention, therefore, consists in a process for producing wool-like or challie effects in cotton fabrics which will not result in damage or material variations in the final product even though variations of wide range occur 60 in the concentration of the acid employed.

It has heretofore been known, also, that 65 wool-like effects may be produced in cotton fabrics by treatment with hydrochloric acid or phosphoric acid or even with nitric acid, but in such cases similar restricted limitations in the range of concentration exist as in the case with sulphuric acid. I 70 have found that sulphuric acid and an inorganic acid, or sulphuric acid and acetic acid, united in determined quantitative proportions produces a mixture having an effect on cotton fabrics different from any of the acids when used alone, that a cotton fabric when treated by such mixture assumed a fine, 75 uniform wool-like or challie character, and that a wide range in variation of the concentration of the acid mixture may occur without material variation in the uniform 80 texture of the resulting product. This permissible wide range of concentration of the mixture is of great importance in furnishing a wider range of control, the elimination to a degree at least of the watchful attention of skilled experts, and lends commercial 85 practicability to the process.

In practicing the process in accordance 90 with the present invention, the cotton fabric may be boiled, bleached and dried, and then mercerized and again dried, or it may be 95 mercerized, then boiled, bleached and dried. In any event, however, it is desirable to remove from the cotton fabric the natural gums and waxes inherent in the fibre and also to remove the sizing placed upon the 95 fabric during the operations following weaving.

The process may be practiced in either 100 mercerized or unmercerized cotton fabric, but preferably the cotton fabric will be mercerized, because such preliminary mercerization causes the cotton yarn to become more even and of uniform texture, while the fabric as a whole is rendered more susceptible to the acid treatment to follow.

In forming the sulphuric and inorganic acid mixture, the inorganic acid may consist of hydrochloric acid or phosphoric acid,

55

60

70

75

80

85

90

95

100

105

each of which has a well-known alterative effect on cotton fibre and of a character different from that of sulphuric acid, and whichever be used, preferably hydrochloric acid, the commercial quality of such acid will be mixed with sulphuric acid in determined proportions. Likewise when a mixture of sulphuric acid and acetic acid is used the commercial quality of acetic acid will be mixed with sulphuric acid in determined proportions.

The acid mixture may vary between 34° Bé. and 42° Bé., and the proportion of sulphuric and hydrochloric acid to produce a mixture of 42° Bé. consists of equal parts of sulphuric and commercial hydrochloric acid, while a mixture of 34° Bé. will be formed of one part of sulphuric acid at 56° Bé. to two parts of commercial hydrochloric acid.

The acid mixture varying from 34° to 42° Bé. produces a uniform, sheer, wool-like finish on the cotton fabric treated by it, notwithstanding the wide range in the acid concentration. The time of the treatment is varied to allow the fabric to undergo the necessary shrinking operation while under the acid treatment.

When the fabric has been treated by acid mixture of a concentration between the limits above stated it may be washed and dried.

What is claimed is:

1. The described process for producing wool-like effects on cotton fabrics which consists in subjecting the fabric to the action of an acid mixture having the property of producing a wool-like effect on the fabric through a range of concentration from 34° to 42° Bé., and consisting of sulphuric acid and a different acid which like the sulphuric acid when used alone has the property of imparting wool-like effects to cotton fabric but at a range of concentration more restricted than the range of said acid mixture.

2. The described process for producing wool-like effects on cotton fabrics, consisting in subjecting the cotton fabrics to the action of an acid mixture of sulphuric acid and hydrochloric acid at a concentration of from 34° to 42° Bé., and then washing the fabrics.

In testimony whereof, I have signed my name to this specification.

HAROLD I. HUEY.